

March 26, 1940.

T. B. CHACE

2,194,738

THERMOSTATIC METAL AND THERMOSTATIC BIMETAL

Filed May 22, 1936



Fig. 1.



Inventor  
Thomas B. Chace  
by Parker & Carter  
Attorneys.

## UNITED STATES PATENT OFFICE

2,194,738

THERMOSTATIC METAL AND THERMO-  
STATIC BIMETALThomas B. Chace, Winnetka, Ill., assignor to The  
Dole Valve Company, Chicago, Ill., a corpora-  
tion of Illinois

Application May 22, 1936, Serial No. 81,284

1 Claim. (Cl. 297—15)

This invention relates to thermostatic metals and bimetals and has for its object to provide a thermostatic metal or thermostatic bimetal which when formed into a thermostatic element will

5 have a useful deflection with temperature change and will particularly have also a high tensile strength and a high resistance to set, so that no change in calibration takes place when the bimetal is incorporated in a device that after use-  
10 ful deflection takes place and further movement of the bimetal is then prevented, the temperature to which the bimetallic element is subjected con-  
tinues to rise, thereby building up considerable force in such element.

15 Tensile strength or resistance to set, as it applies here, of a solid-solution-type alloy is first the result of chemical analysis. Variables of these properties are relative to hardness, and hardness is relative to wrought or work hard-  
20 ening. The present thermostatic bimetal applica-  
tions require severe forming of the elements to incorporate them in thermostat devices. I have found that if the now available thermostatic bimetals are hardened by working, such as roll-  
25 ing to the extent that resistance to set is high, they are too refractory and fracture in forming, which fracture becomes the weakest point and destroys the resistance to set. If work hardened only sufficiently to be ductile enough for form-  
30 ing, the resistance to set is low.

Invar or the low expanding nickel alloy has a higher modulus of elasticity than the copper alloys in similar work hardened condition and one object of this invention is to provide a bi-  
35 metal element of Invar and a copper alloy which copper alloy has a similar modulus of elasticity to Invar. The invention may be used in any de-  
sired manner where thermostatic metal is de-  
sirable.

40 A particular application of the invention is automobile cooling system thermostats incorporating a movable valve for controlling water flow and a temperature responsive bimetal coil element which is arranged in a coil or otherwise, to move the valve to its open and closed position. For purposes of illustration I have indicated in the drawing one form of device illustrating such use.

50 Fig. 1 is a view in part section, showing an automobile cooling system with a valve and thermostat in position;

Fig. 2 is an enlarged sectional view through the casing of the valve and thermostat;

55 Fig. 3 is a sectional view through the valve

casing, taken on line 3—3 of Fig. 2, showing the entire valve.

Like numerals refer to like parts throughout the several figures.

In this construction there is a valve 1 arranged in a casing 1a, the valve and casing being located in the pipe 2 leading from the engine jacket 3 to the radiator 4. I have illustrated a stop 5 which is engaged by the valve when the valve is in its fully open position, as shown in dotted lines in Figs. 1 and 2. When the engine is cold the valve is closed, as shown in full lines, and when the cooling liquid for the engine heats up, the thermostat is heated and moves the valve to its open position. In this use in its action through 15 the temperature range of approximately 140° to 180° F., the bimetal element has completed its useful deflection and the valve has reached its wide open position, as shown in dotted lines in the drawing, so no further travel is necessary or 20 possible. Temperatures greatly in excess of 180° F. are sometimes reached in an automobile cooling system due to low water, frozen radiator, or numerous other causes. Any increase in tem-  
25 perature over 180° F. builds up a force in the bi-  
metal element, which if free would continue to deflect with temperature increases. Since the valve 1 cannot move any farther than to its fully open position, as shown in dotted lines, its move-  
30 ment is stopped and the increase in temperature simply builds up a force in this thermostatic ele-  
ment without producing any further movement of the valve 1. If the element does not have a high resistance to set, under this condition a change in calibration takes place increasing the operat-  
35 ing range above the original 140° to 180° F., causing continual overheating and possible se-  
vere damage to the engine.

I have provided a thermostatic bimetal entirely satisfactory for this type of application by 40 utilizing with a low expanding member, such member formed of nickel and iron containing 32 to 45 percent nickel and remainder iron, a copper alloy having a relatively high and cooper-  
45 ating co-efficient of expansion and other prop-  
erties permitting a combination of the nickel steel alloy and the copper alloy of approximate-  
ly equal proportional thickness in composite slab form to be converted into sheet form. This copper alloy has the important property of harden-  
ing without working or reduction of area so that the completely formed bimetal element as ready 50 for assembly into the device can be further hard-  
ened and resistance to set increased by aging.

I provide a copper alloy, which of the solid 55

solution type, has a relatively high modulus of elasticity and to this I add an element or combination of elements, the solubility of which in the copper alloy is greater at high temperatures than at low temperatures.

Age hardening, or precipitation hardening occurs only in alloys of the solid solution type which contain a hardening constituent, the solubility of which in the alloy at high temperatures is greater than at low temperatures. The solid solution when quenched from the above solid solubility temperature is supersaturated and unstable and on reheating to a temperature below the solid solubility temperature, the unstable solution tends to revert to an equilibrium condition which corresponds with a tempering effect. The resulting increase in hardness is a supersaturated solid solution hardening.

Usually increases in hardness and strength or resistance to set are comparable and this is true of the alloy covered here for thermostatic bimetal.

There is a change with temperature in the solubility of iron in copper from approximately 4 percent at 2000° F. to approximately .5 percent at 1000° F. I find that iron as a hardening constituent in my copper alloy for thermostatic metal use to be particularly desirable, as drastic quenching is not necessary to bring about supersaturation at low temperatures. Remarkable hardening can be produced by cooling slowly and reheating to a temperature under the first temperature. The solubility of silicon in copper varies from 6.7 percent at 1350° F. to about 4 percent at 750° F. but a copper alloy containing over 3 percent silicon is very refractory and difficult to roll. So silicon alone as a hardening constituent is not desirable. However, silicon with necessary amounts of nickel and iron, forming the corresponding silicides are particularly susceptible to age hardening; for example, nickel silicide is soluble in copper to the extent of 8.2 percent at 1830° F. and only .7 percent at 570° F. I have found that a nickel-iron-silicon-manganese-copper alloy having the metals in substantially the following proportions to be particularly useful and efficient for my thermostatic bimetal, nickel .5 percent to 5 percent, iron .1 percent to 5 percent, silicon .5 percent to 3 percent, manganese .25 percent to 1 percent, and the remainder copper.

The thermostatic bimetal of Invar and the

silicon - nickel - manganese - iron - copper alloy above set out for this purpose are welded in slab form and rolled into sheet or strip. This is cut up into usable sizes and then formed into coils or other shapes and then treated to increase resistance to set.

The resulting strength of the bimetal element after treating is greater than that obtained by work hardening as by cold rolling to a hardness which is still ductile enough for forming into a coil shape like the automobile cooling system thermostatic coil.

Hardening of the foregoing age hardenable alloy is done by heating to approximately the solid solution temperature of the particular alloy and then quenching. The hardening or aging takes place during a subsequent reheating of one to several hours to a temperature lower than the quenching temperature. The quenching temperature is usually between 1300° F. and 1600° F. and the aging temperature between 400° F. and 1150° F. When temperature and time prior to quenching are sufficient to anneal or soften the Invar, the following increase in hardness by aging the copper alloy would in some combinations not be as great as the loss and the bimetal shape would have a lower resistance to set than before age hardening. In this event, the first heating and quenching is done prior to the finished gauge thickness and then cold worked by rolling to harden the Invar, which work hardens more readily than the copper alloy. The copper alloy is partially hardened by the cold working but only sufficiently so as to be ductile enough for forming. Further hardening is then accomplished on the formed or shaped individual bimetal coils or pieces by aging at a temperature lower than the quenching temperature. The resulting increased hardness of the copper alloy is similar to the effect from excessive cold working but if hardened in sheet form by cold rolling the material would not form, as described, without fracture.

I claim:

A thermostatic bimetallic element having a member formed of a ferrous alloy comprising 35 percent to 45 percent nickel and a member formed of a copper alloy comprising silicon 0.5 percent to 3.0 percent, nickel 0.5 percent to 5.0 percent, manganese .25 percent to 1.0 percent, iron 0.1 percent to 5.0 percent, and the remainder copper.

THOMAS B. CHACE.